

March 13, 1951

G. S. GIBBS

2,545,352

METHOD OF MAKING RAISED ELECTRICAL CONTACT POINTS

Filed Aug. 5, 1947



Fig. 6.



Inventors:

George S. Gibbs

By James R. Hodder

Attorney

## UNITED STATES PATENT OFFICE

2,545,352

METHOD OF MAKING RAISED ELECTRICAL  
CONTACT POINTS

George S. Gibbs, Newton, Mass.

Application August 5, 1947, Serial No. 766,336

2 Claims. (Cl. 29—155.55)

1

My present invention is a novel and improved method of manufacturing various articles utilizing powdered metal under heat and pressure, and is particularly valuable in making electrical contact points, ornamentations for jewelry, and the like.

My invention is especially applicable to the manufacture of articles utilizing powdered silver, and comprises improved methods of handling such powdered metal, conserving the quantity of powder necessary in the making of any specific article, insuring uniformity in successive articles and utilizing a novel and improved continuous method of manufacture.

Heretofore it has been customary in the making of electrical contact devices, for example, to utilize silver for the contact points, first forming the silver article into a disc by cutting from a sheet of such metal, or otherwise. Cut and formed base material was utilized with protuberances in which the metal discs were applied, usually by hand, and soldered in place in a furnace, after which the base material was re-struck or coined, thus forcing the metal discs to conform to the protuberances in the base metal, resulting in a protuberance capped with silver for better operation.

Such discs and the positioning of the same on the base material was subject to considerable error and displacement in position, so that the resultant contact elements cut from the sheet comprising two, three, or more of such contacts lacked uniformity, and also caused unnecessary flow of added material (silver) at the periphery of the protuberance.

In my present invention I utilize a powdered metal, such as silver, for the contact points or for the ornamentation desired in jewelry manufacture, and first make the indentations in the base material and then apply a small quantity of the powdered silver into the said indentations, first coating the indentations with a suitable flux to permit the powder to be bonded to the base when sintered and solidified in permanent bond with the base material. Thereupon, after the waste powder has been swept or struck from the top of the indentation and sintered or solidified, the under or reverse side of the base material is punched upwardly or indented from the bottom, thus forming the metal surface in a rounded projecting position for electrical contact use, jewelry ornamentation, or other purposes.

Thus my method enables the powdered silver to be accurately positioned with rounded uniformity to utilize a minimum quantity of the sil-

2

ver powder and to result in a better union of the powdered metal under heat and pressure during the sintering operation and, thus, giving a more permanent bond and union in the fusing of the flux element with the base material, as well as uniformity in the resultant article made thereby.

In as expensive a material as powdered silver, the saving in the powder itself for such contact points as above described is of great importance and the operation of first indenting a sheet of metal as a base insures the location and position of the silver applied to such indentations. The coining operation also is accurately and effectively performed. Also, my method results in presenting the thickest coating of silver at the crown of the protuberance, and thinning out around the periphery—thus increasing wear-resistance at the crown.

While I prefer to first intent the base, then to apply a coating or fluxing element, and thereafter to supply the powdered silver to the indentations, I may utilize the powdered material with the fluxing element mixed therein and, thus, supply both during the action of filling the indentations. Or I may utilize the powder with or without the fluxing element as a portion of the indenting action. Thereafter, the sintering operation gives a firm bond and union between the powdered silver and the base metal as well also as solidifying the powder into a uniform mass. Thereafter, the punching upwardly of the base metal under each of the silver coated points effects the raising and projecting of the silvered parts into operative or ornamental position, with maximum material at the top of the projection and minimum at the periphery of the projection. Also, I may simply recess the base material and fill the same with powdered metal or silver, compacting it in any desired way, and this feature I wish to claim herein broadly.

Referring to the drawings illustrating my preferred method of manufacture and improved article made thereby:

Fig. 1 is a diagrammatic view showing a continuous method of operation;

Fig. 2 is an enlarged cross-sectional view of one of the powder-receiving depressions made in the base metal;

Fig. 3 illustrates the filling of such a depression with powder;

Fig. 4 is illustrative of the fusing, solidifying, and sintering of the powdered metal in the depression;

Fig. 5 is a diagrammatic view of the punching operation forming the previously indented surface

55

into a projecting position on the base plate; and

Fig. 6 is a fragmentary view of the base with a plurality of depressions for receiving the powdered metal.

Referring to Fig. 1, a coil or roll of suitable base material is indicated at 1, which material is fed thru a pair of feed rolls 2 and 3 at appropriate speed, feeding the strip 1 into and thru a stamping press 5, wherein a row of indentations as indicated at 6 is stamped crosswise of the metal base 1. The stamped base with the recess 6 is thereupon fed thru a station 8 which applies a fluxing element 10, see Fig. 2, as a coating or the like into each of the depressions 6. Thereafter, the continuous travel of the base 1 carries the same with the depressions uppermost by a powder filling station 12, which will flow a suitable amount of powdered silver into each of the depressions 6 on top of the flux coating 10. Thereupon, the base 1 passes by a scraping or cleaning operation, wherein a series of brushes or the like, as indicated at 14, will strike off surplus powder from the depressions 6, leaving the powder as shown at 15, Fig. 3, flush or level with the top of the base 1.

Continued travel of the strip 1 carries the same with the powder in the depressions thru a sintering furnace 20, which thereupon solidifies the powder 15 into a compact mass as indicated at 21, Fig. 4, acts on the flexing element to thereby effectually bonding and uniting the solidified powder and the base, which, by this operation would normally be slightly depressed below the level of the top of the plate 1 at each depression. A cooling tunnel is indicated at 24 so that the continued line of travel of the base 1 with the sintered powder and base thus united will be sufficiently cooled and set for subsequent handling.

I find it desirable to have a slack control which is indicated at 25 in advance of the feed rollers 26 and 27 so that the base 1 may be momentarily held against continuous feeding motion during the punching of the recesses, supplying the fluxing element and powder to the recesses; whereupon the base 1 continues its line of travel to a second stamping press 30, which effects a reverse punching operation of the recesses 6, punching the same into a projecting recess 3 on the opposite side, thus elevating the solidified silver surface 35 into a raised position, as shown at Fig. 5. This stamping press would simultaneously coin,

form, and cut off predetermined shapes or sections from the strip 1, as indicated at 36; whereupon these sections would travel down the chute 38 and be collected into a receptacle 40. Thus, 5 raised silver surfaced projections or bosses are readily and accurately positioned and produced automatically, and at great speed, entirely independent of manual handling and spotting of discs, as well as without the skilled labor previously required.

I claim:

1. The method of forming a raised electrical metallic contact point with metallic backing material, which consists in indenting a metal base sheet, applying a coating of flux to the surface of the indentation, filling the indentation with metal powder, heating the metal powder and the base sheet to sinter the metal powders together and to bond the sintered metal powder to the base sheet, and then re-indenting the base sheet from the opposite surface to produce a raised electrical contacting point.

2. The method of forming a raised electrical metallic contact point with metallic backing material, which consists in indenting a metal base sheet, applying a coating of flux to the surface of the indentation, filling the indentation with silver powder, heating the silver powder and the base sheet to sinter the silver powders together and to bond the sintered silver powder to the base sheet, and then re-indenting the base sheet from the opposite surface to produce a raised electrical contacting point.

GEORGE S. GIBBS.

#### REFERENCES CITED

The following references are of record in the file of this patent:

#### UNITED STATES PATENTS

| Number    | Name        | Date          |
|-----------|-------------|---------------|
| 1,046,823 | McBerty     | Dec. 10, 1912 |
| 1,744,810 | Shallcross  | Jan. 28, 1930 |
| 2,137,617 | Imes et al. | Nov. 22, 1938 |
| 2,181,083 | Payette     | Nov. 21, 1939 |
| 2,365,249 | Comstock    | Dec. 19, 1944 |
| 2,390,595 | Larsen      | Dec. 11, 1945 |
| 2,417,967 | Booe        | Mar. 25, 1947 |
| 2,425,053 | Swinehart   | Aug. 5, 1947  |
| 2,458,552 | Blattner    | Jan. 11, 1949 |
| 2,473,371 | Heath       | June 14, 1949 |